

April 23, 1957

**J. WALLERIUS** 2,789,  
PROCESS OF HARDENING STEEL CARTRIDGE CASES AND APPARATUS  
FOR ACCOMPLISHING SUCH PROCESS

2,789,928

Filed July 1, 1952

7 Sheets-Sheet 1



INVENTOR.  
*John Wallerius*

BY  
McLennan & Morlach

Attys

April 23, 1957

J. WALLERIUS

**2,789,928**

PROCESS OF HARDENING STEEL CARTRIDGE CASES AND APPARATUS  
FOR ACCOMPLISHING SUCH PROCESS

Filed July 1, 1952

7 Sheets-Sheet 2



*INVENTOR.*

John Wallerius

BY  
McGraw & Morsbach

Attys.

April 23, 1957

3, 1957 J. WALLERIUS 2,789  
PROCESS OF HARDENING STEEL CARTRIDGE CASES AND APPARATUS  
FOR ACCOMPLISHING SUCH PROCESS

2,789,928

Filed July 1, 1952

7 Sheets-Sheet 3



April 23, 1957

J. WALLERIUS 2,789,928  
PROCESS OF HARDENING STEEL CARTRIDGE CASES AND APPARATUS  
FOR ACCOMPLISHING SUCH PROCESS

Filed July 1, 1952

7 Sheets-Sheet 4

FIG 9



FIG 8



FIG 10



INVENTOR.

John Wallerius

BY  
McLenna & Morslach

Atty's

April 23, 1957

J. WALLERIUS  
PROCESS OF HARDENING STEEL CARTRIDGE CASES AND APPARATUS  
FOR ACCOMPLISHING SUCH PROCESS

2,789,928

Filed July 1, 1952

7 Sheets-Sheet 5

FIG. 14



FIG. 15



FIG. 11



20

FIG. 12



INVENTOR.  
John Wallerius

BY  
McGraw & Morelack

Atty.

April 23, 1957

**J. WALLERIUS** 2,789,  
PROCESS OF HARDENING STEEL CARTRIDGE CASES AND APPARATUS  
FOR ACCOMPLISHING SUCH PROCESS

2,789,928

Filed July 1, 1952

7 Sheets-Sheet 6



FIG. 13a

*INVENTOR.*

John Wallerius

BY  
McLennan & Moorebach  
Attns.

April 23, 1957

J. WALLERIUS

2,789,928

PROCESS OF HARDENING STEEL CARTRIDGE CASES AND APPARATUS  
FOR ACCOMPLISHING SUCH PROCESS

Filed July 1, 1952

7 Sheets-Sheet 7



FIG. 13b

*INVENTOR.*

John Wallerius

BY  
McAnna & Morsbach

Attys.

# United States Patent Office

2,789,928

Patented Apr. 23, 1957

1

2,789,928

## PROCESS OF HARDENING STEEL CARTRIDGE CASES AND APPARATUS FOR ACCOMPLISHING SUCH PROCESS

John Wallerius, Glen Ellyn, Ill., assignor to Sunbeam Corporation, Chicago, Ill., a corporation of Illinois

Application July 1, 1952, Serial No. 296,595

12 Claims. (Cl. 148—13)

The present invention relates to a method and apparatus for hardening steel cartridge cases, and more particularly small caliber steel cartridge cases.

Heretofore cartridge cases have been formed primarily from brass, which is a resilient material capable of expanding and contracting almost instantaneously. Such brass cartridge cases were manufactured in quantity and were heat treated by moving the cartridges through a furnace in random fashion, as by being disposed in random fashion on a movable conveyor of some sort. For numerous reasons, including among them the shortages of copper, cartridge cases have recently been made of steel. It has been discovered that steel cartridge cases present a much more difficult heat treating problem than brass cartridge cases. In the first place, if the steel is too hard, it will not expand as it should within the gun barrel upon firing of the cartridge, and the cartridge case breaks in the gun. On the other hand, if the steel cartridge case is not hard enough, it expands very rapidly but will not contract, and then tends to stick in the gun. Moreover it has been found that uniform hardness around the entire base of the cartridge case is essential and there must not be hard and soft spots. To obtain such uniform hardness, a critical heat treating process is essential, and random heating, as heretofore employed and satisfactory in connection with brass cartridge cases, will not be satisfactory. It has been found in connection with the present invention that the cartridge cases must be moved through the hardening furnace, all orientated in exactly the same way to insure uniform hardness, and immediately upon leaving the furnace the cartridge cases must be quenched uniformly and very rapidly to obtain the desired hardness. The importance of this quench may be better appreciated when it is considered that the temperature of the cartridge cases, which reaches a maximum of something over 1600° F., must be reduced to room temperature in a matter of a few seconds, which means that the quenching apparatus must almost be inside the furnace. By accurately controlling the hardness of such steel cartridge cases, it is possible to hold to closer size tolerances, with greatly improved surface qualities of the cartridge cases. Moreover, the quality of the heat treating has been found to have a direct effect on the number of acceptable cartridges cases produced.

It will readily be understood that to reduce the temperature in a matter of a few seconds from a high heat treating temperature to room temperature or below in a continuous furnace capable of producing thousands of cartridge cases in an hour, requires a rather unusual quenching device, and one of the features of the present invention resides in an improved quenching device.

As will become apparent from the ensuing description, in order to insure uniform heating every cartridge case must be moved through the furnace in the same way, in other words orientated in the same way, and this is accomplished in accordance with the present in-

2

vention by pushing the cartridge cases in end-to-end relationship through suitable heating tubes within the furnace. The forward end of one cartridge case will then engage the base of the preceding cartridge case. Obviously, at the high temperatures to which these cases are subjected within the furnace, there will tend to be welding together of the engaging portions of the adjacent cartridge cases. It would be desirable to provide an arrangement whereby such welding together of the adjacent cases will in no way interfere with satisfactory operation.

Accordingly, it is an object of the present invention to provide a new and improved method for heat treating steel cartridge cases to insure uniform hardness to a desired extent.

It is another object of the present invention to provide an improved heat treating furnace for heat treating steel cartridge cases to the same uniform hardness.

It is another object of the present invention to provide an improved furnace for heat treating steel cartridge cases wherein such cases move through the furnace, all orientated in exactly the same fashion, and wherein such cases are quenched to reduce the temperature thereof greatly within a matter of seconds after leaving the furnace atmosphere.

It is a further object of the present invention to provide an improved quenching apparatus for a heat treating furnace wherein cartridge cases move through the furnace with many cartridge cases being discharged every fraction of a minute, which will simultaneously quench the inside and outside surfaces of the successive cases as they are discharged from the furnace.

A further object of the present invention resides in an improved ejection device for ejecting quenched cartridge cases, using air under pressure directed toward the interior of the cartridge case to eject the same from the quenching device.

Still another object of the present invention resides in an improved control system for an automatic continuous heat treating furnace which insures a continuous supply of cartridge cases to the furnace, uniform heating of all the cartridge cases as moved through the furnace, rapid quenching immediately upon completing the pass through the furnace, and ejection of the quenched cartridge cases in a matter of a few seconds after the quenching operation is initiated.

Another object of the present invention resides in the use of a noncorrosive quenching liquid in connection with a heat treating furnace employing a suitable wetting agent whereby high speed quenching operation is obtained without the corrosive effect of brine quenches heretofore used.

A still further object of the present invention resides in simple static means for periodically causing movement of the individual cartridge cases transversely to their direction of movement through the furnace to eliminate the possibility of welding together of engaging portions of adjacent cases.

Further objects and advantages of the present invention will become apparent as the following description proceeds, and the features of novelty which characterize the invention will be pointed out with particularity in the claims annexed to and forming a part of this specification.

For a better understanding of the present invention, reference may be had to the accompanying drawings in which:

Figs. 1 and 2 together comprise a sectional view through the entire furnace of the present invention, with Fig. 1 showing the feed end of the furnace, and Fig. 2 showing the discharge and quenching end of the furnace;

Fig. 3 is a partial sectional view taken along line

3—3 of Fig. 1, and assuming that Fig. 1 shows the complete structure;

Fig. 4 is an enlarged view, partly in section looking in the direction of the arrows 4—4 of Fig. 3;

Fig. 5 is an enlarged sectional view taken along line 5 5—5 of Fig. 1, assuming that Fig. 1 shows the complete structure;

Fig. 6 is an enlarged sectional view of a portion of Fig. 1 to illustrate more clearly the movement of the cartridge cases through the furnace;

Fig. 7 is an enlarged sectional view taken along line 7—7 of Fig. 2, assuming that Fig. 2 shows the complete structure;

Fig. 8 is an enlarged sectional view of a portion of the quenching apparatus shown in Fig. 2 of the drawings; 15

Fig. 9 is a sectional view taken along line 9—9 of Fig. 8, assuming that Fig. 8 shows the complete structure;

Fig. 10 is a sectional view taken along line 10—10 of Fig. 8, again assuming that Fig. 8 shows the complete 20 structure;

Fig. 11 is an enlarged view of the feeding apparatus shown in Figs. 1 and 3, and preferably taken along line 11—11 of Fig. 3;

Fig. 12 is a sectional view taken on line 12—12 of Fig. 1 of about one-half of the furnace; 25

Figs. 13a and 13b together comprise a complete control circuit, including a schematic disclosure of the elements controlled;

Fig. 14 is an enlarged sectional view illustrating a 30 modification of the present invention; and

Fig. 15 is a sectional view of reduced size taken along line 15—15 of Fig. 14, assuming that Fig. 14 shows the complete structure.

Briefly, the present invention is concerned with a heat treating furnace in which steel cartridge cases are pushed in end-to-end engagement through tubes extending through a heat treating furnace. A large number of tubes may be employed in parallel, and preferably the tubes contain cracked city gas or another suitable non-oxidizing medium to reduce scaling and the formation of oxides. Automatic means are provided for simultaneously pushing a new cartridge case into each of the parallel tubes, and simultaneously pushing along all the cartridge cases within the tubes. A feeding mechanism is provided to permit automatic feeding of cases to the entrance to each of the tubes. In effect, the cartridge cases are "walked" through the tubes to prevent welding of engaging cartridge cases. At the discharge end of the furnace the cartridge cases fall by gravity through an external quenching jet into a receiving cage and while therein are immediately subjected to an internal jet of a very cold noncorrosive quenching liquid to reduce the temperature from something over 1600° F. to room temperature in a matter of a few seconds. A few seconds later, the receiving cage into which these cartridge cases are ejected for quenching moves to an ejecting position, and a stream of air literally blows the cartridge cases out of the quenching cage and into a wash tank. A suitable control circuit is provided, controlled by a cycle timer which determines the speed of the heat treating cycle. Full automatic control is provided.

Referring now to the drawings, and primarily to the structural disclosures of Figs. 1 to 12, inclusive, there is provided a main furnace structure generally designated by the reference numeral 20 comprising an elongated heating section which may have any cross sectional configuration but which preferably is of rectangular external configuration. There is defined within the furnace a heating chamber generally designated at 22 which extends from end to end of the furnace and which is preferably defined by a layer of insulating fire brick 23 on the top, a layer of insulating fire brick 24 on the bottom, and similar layers of insulating brick 25 and 26 at each end, as well as a layer 27 along each side. Sur-

rounding the insulating fire brick is preferably a layer of insulating brick 28, and around the insulating brick is preferably a layer of loose asbestos 29, the latter of which is enclosed by a suitable steel shell 30, the various layers of insulation taking care of the temperature gradient from inside of the furnace, which is of the order of 1650° F. for a particular heat treating operation, to room temperature at the outside of the furnace. Preferably the insulating fire brick is capable of withstanding temperatures up to 2600° F., the insulating brick 28 is capable of withstanding temperatures up to 1600° F., and the loose asbestos 29 is capable of withstanding temperatures up to 800° F.

For the purpose of supporting the means defining the heating chamber 22, at a suitable height, there is provided a suitable frame of channel members, angle irons and the like, generally designated by the reference numeral 32, the particular construction of which forms no part of the present invention. To simplify the support means, the top of the heating chamber 22 is arched as indicated at 33, thereby inherently providing support. This is best shown in Fig. 12 of the drawings.

Any suitable means for supplying heat to the furnace, such as a source of gas heat or electrical heat, may be employed. Preferably, and in accordance with the present invention, electrical resistors are used to supply the heat within the furnace chamber 22, and these electrical resistors not shown are preferably disposed along the interior walls of the furnace chamber 22, such as along the arched top 33 thereof as well as along the floor of the furnace.

To insure that the cartridge cases are all orientated in the same manner in passing through the heating chamber 22, there are disposed within the heating chamber 22 a 35 plurality of elongated tubes 36 arranged in spaced parallel relationship. The particular number of tubes employed is immaterial as far as the present invention is concerned, and in Fig. 3 of the drawings twenty-four tubes 36, arranged in a common plane in spaced parallel relationship, are shown. These tubes are preferably formed of a suitable alloy material capable of withstanding the high temperatures produced in heating chamber 22. For 40 the purpose of supporting the tubes 36 in spaced parallel relationship within the heating chamber 22, fire brick piers 34 are provided, upon which are disposed suitable alloy pier caps, upon which in turn are mounted suitable tube supports 35 formed of a heat resisting alloy. These tube supports 35 are preferably provided with suitable slots to appropriately space the tubes. A second spacer member 35a is disposed on the top of the tubes and suitably locked to supports 35, whereby the tubes 36 are supported as a unitary structure within the chamber 22. The feed end of the furnace is shown in Fig. 1, and the tubes 36 protrude from this feed end through suitable 45 openings defined in the furnace wall. The protruding ends of the tubes 36 are provided with flared ends 37 to facilitate the entrance of the cartridge cases by automatic means described in greater detail hereinafter.

It will be apparent that if steel cartridge cases are subjected to a high temperature in an ordinary atmosphere which is at all oxidizing in nature, a great deal of scaling and oxidation will occur. In accordance with the present invention, a nonoxidizing atmosphere is preferably maintained within the tubes 36, and to this end a suitable 50 controlled atmosphere, such as cracked city gas, is supplied from a header 39 through conduits 40 into the alloy tubes 36. For the purpose of insuring that the nonoxidizing atmosphere supplied through the conduits 40 is at a raised temperature when entering the alloy tubes 36, the conduits 40 preferably extend for a substantial distance within the heating chamber 22 before entering the tubes 36. This atmosphere escapes from the flared ends 37 of the tubes 36 and is burned at the feed end of these tubes so that across the feed end of all of the tubes 55 78 36, best shown in Fig. 3, gas flames will appear thereby

preventing the entrance of an oxidizing atmosphere. The atmosphere within the tubes 36 is an endothermic gas, preferably obtained by applying heat to crack ordinary city gas with air. This results in a gas comprising 20% carbon monoxide, 40% hydrogen, and 40% nitrogen.

It will be understood by those skilled in the art that cartridge cases have relatively thin walls, and at the high temperatures encountered within the heating chamber 22 the walls of the cartridge cases tend to soften. It is, however, essential that no distortion of the walls of the cartridge cases occurs, and in accordance with the present invention the tubes 36 have a particular configuration for distributing the weight of the cartridge cases in movement therethrough. This is best shown in Fig. 5 of the drawings, which is a section through one of the tubes 36 and indicates that the lower portion of the tubes 36 has a somewhat V-shaped configuration. A cartridge case, generally designated by the reference numeral 42, is shown disposed within the cross section of the tube 36, and it is obvious that with the V-shaped configuration the cartridge case is supported at 43 and 44, thereby tending to distribute the weight of the cartridge case. If the tubes 36 had a circular configuration, it is apparent that the cartridge case would engage the same only along a line at the bottom of the tubes 36 and the cartridge cases 42, and much more likelihood of distortion of the thin walls of the cartridge cases at high temperatures might occur.

From the discussion above it will be understood that the cartridge cases are effectively pushed through the tubes 36, each succeeding cartridge case in effect being an inserted force transmitting member for transmitting force from a suitable pusher device to be described hereinafter to successive cartridge cases disposed within the tubes 36. The end-to-end relationship of the cartridge cases 42 is shown in dotted lines within the tubes 36 in Figs. 1 and 6 of the drawings. At temperatures as high as 1600° F. the engaging ends of the cartridge cases 42 may tend to weld together, and this is particularly true with respect to the engaging surface of two adjacent cartridge cases when making the complete pass through the tubes 36 within heating chamber 22. To prevent this, in accordance with the present invention, the cartridge cases 42 are effectively "walked" through the tubes 36, which is another important feature of the present invention. At closely spaced intervals, which may be of the order of every 8 inches, the apex of the V-shaped bottom of the tubes 36 is indented to provide inwardly extending protuberances 46 which cause the cartridge cases to raise and lower slightly in a direction transverse to the general direction of movement through the tubes 36. This transverse movement, which first tips one end of the cartridge case upwardly (see Fig. 6) and then tips the other end of the cartridge case upwardly, effectively keeps breaking any welding which might occur at the engaging ends of adjacent cartridge cases.

From the above description the movement of the cartridge cases 42, beginning with movement upon insertion into the flared openings 37, along the tubes 36 will be apparent, and consideration now will be given to the discharge of the cartridge cases from the discharge ends of the tubes 36 shown in Fig. 2 of the drawings. Each of the tubes 36 terminates in a somewhat enlarged chamber designated as 50, which is connected to a discharge chute 51, one being provided for each tube 36. The chutes 51 each have a sort of enlarged funnel-shaped portion where connected to the discharge end of the associated tube 36. Each discharge chute 51 has the same V-shaped configuration as the tubes 36 (see Fig. 10 of the drawings) and extends through a suitable opening 52 defined in the furnace 20. Adjacent where the discharge chute 51 is connected to the tubes 36, there is provided a suitable observation opening connected by a tube 54 which extends outside the furnace. The end of the tube is closed by a suitable observation cover or sight glass so that one may view the

discharge end of each tube 36. The two end tubes 36 adjacent the two sides of the furnace, and specifically designated as 36a and 36b in Fig. 3 of the drawings, are provided adjacent the discharge ends of the tubes with lateral openings 55 (it is assumed that the particular tube 36 visible in Fig. 2 of the drawings is the tube at the extreme end, namely, tube 36a), which is also connected by a suitable tube to a suitable sight glass to permit observation of the cartridge cases moving through the particular tubes such as 36a, which will, of course, be representative of what occurs in the other tubes 36 not provided with such sight glasses.

From an examination of Fig. 2 of the drawings it will be noted that there is illustrated a cartridge case 42 which has just fallen into the discharge chute 51, and the next case 42 is almost ready to fall into the discharge chute 51, it having just passed the last protuberance 46. In the event that the hardening furnace 20 were shut down over the week-end, for example, with this last cartridge case in the position shown in the drawings, it is possible that this cartridge case might be welded to the engaging end of the cartridge case immediately behind it, and in that case pushing in new cartridge cases from the other end might tend to jam the last cartridge case against the end wall of the tube defined by the discharge chute 51. In accordance with the present invention, a suitable wedge-shaped member 58 is provided above the discharge chute 51 to deflect the last cartridge case 42 in the event that it is welded to the succeeding cartridge case. It will be understood that the wedge-shaped member 58 is only employed following shutdown of the furnace, since normally the protuberances 46 will prevent such welding operation, and the cartridge case 42 which moves into the discharge chute 51 will tend to drop by gravity before engaging the wedge-shaped member 58. However, this member is provided as a safety feature in the event that for any reason the protuberances 46 do not function to prevent such welding operation of adjacent cartridge cases.

The endothermic gas or noncorrosive atmosphere supplied by the conduits 40 to the tubes 36 must not escape from the end of the discharge chute 51, and yet this discharge chute must be open to permit cartridge cases 42 to drop out by gravity. In accordance with the present invention and as best shown in Figs. 2 and 8 of the drawings, the end of discharge chute 51 is provided with a short jacket 60 which defines an annular chamber 61, which chamber is preferably connected by a suitable conduit 62 with a cooling or quenching liquid described in greater detail hereinafter. The end of the discharge chute 51 and the corresponding end of the jacket 60 are so constructed as to define a somewhat annular nozzle 63. This annular nozzle is designed to discharge an annular stream of quench liquid converging at a point and consequently in effect discharging a somewhat cone-shaped wall of liquid designated at 64 in Fig. 8 of the drawings. This cone-shaped wall of liquid closes the end of the discharge chute 51 as far as the escape of any of the endothermic gas or noncorrosive atmosphere contained therein is concerned, and yet the cartridge cases 42 may be discharged through this wall of quenching liquid, which, therefore, in effect performs two functions: one, it prevents the escape of the atmosphere contained within the tubes 36, and two, it provides an external liquid quench for cooling the cartridge cases 42, which second function will be described in greater detail hereinafter. Preferably the discharge chutes 51 are provided with openings 67, to which are connected suitable conduits 68 which may be connected to a manifold 69, which manifold may be provided with suitable openings at which the cracked city gas may be burned, preferably at a point which will not interfere with personnel working near the furnace. Unfortunately, there is no way that this can be accomplished at the feed end of the tubes 36 and, hence, the gas must be burned at the feed opening in each of the tubes.

In order to understand the automatic feeding of car-

tridge cases to the flared ends 37 of the tubes 36, reference may be had to Figs. 1, 3, 4 and 11 of the drawings. At the feed end of the furnace there is provided a loading and feeding unit generally designated by the reference numeral 70. This loading and feeding unit comprises an endless roller chain conveyor 71, mounted for rotation about relatively large diameter spaced sprockets 72 suitably journaled adjacent each end of a support in the form of a framework 73 extending across the feed end of the furnace 20 and including a portion 73a extending to one side of the furnace defining a loading table described hereinafter. Attached to the outside of the roller chain conveyor 71, as best shown in Fig. 4 of the drawings, as by suitable fastening means 76, are a series of elongated U-shaped cartridge case receptacles 75 uniformly spaced along the roller chain 71 in the same manner as the tubes 36 are spaced, and of a size capable of receiving therein a single cartridge case with its longitudinal axis transverse to direction of movement of the roller chain 71. It will be apparent that the endless chain 71 is in effect an endless magazine having its upper flight positioned so the cartridge case receptacles 75 are on a level with the flared openings 37 in the tubes 36. If the endless magazine is stopped in a position so that each receptacle 75 is exactly opposite a corresponding flared opening 37, a suitable end thrust on the cartridge cases disposed in the magazine will move them directly into the flared openings 37. The portion of the endless magazine extending laterally of the furnace 20 furnishes a loading zone for the magazine sufficiently removed from the gas flames at the openings 37 to permit personnel to load the same. It is essential that the receptacles 75 in front of the openings 37 be maintained level, and to this end horizontally disposed angle iron supports 78 disposed on the frame 73 eliminate and sag in the upper flight of roller chain 71.

For the purpose of moving the cartridge cases disposed in the receptacles 75 when the receptacles are moved into alignment with the ends of the tubes 36, there is provided a suitable pusher mechanism generally indicated at 79 and comprising a plurality of spaced fingers 80 mounted on a common angle-shaped support 80a, which latter is connected by a suitable connecting rod 81 to a fluid motor 84 comprising a piston 82 reciprocally mounted in a cylinder 83, best shown in the schematic diagram of Figs. 13a and 13b. The ends of the support 80a are preferably attached to suitable rollers 86, mounted for movement on spaced guideways 87, whereby guided reciprocal movement of the fingers 80 can occur in response to operation of fluid motor 84. Preferably a hydraulic motor is used for causing operation of the pusher mechanism 79, although it should be understood that any other prime mover may be employed. As best shown in Figs. 13a and 13b of the drawings, a solenoid actuated valve 88 controls the operation of the fluid motor 84. Preferably the solenoid valve 88 controls movement in each direction of the piston 82. For the purpose of simplifying the drawings, however, in Figs. 13a and 13b the fluid motor 84 has been shown as a spring return fluid motor, whereby upon energization of the solenoid valve 88 the piston 82 moves toward the right, as viewed in Figs. 13a and 13b, under the pressure of the hydraulic fluid, and upon deenergization of the solenoid valve 88 the piston 82 moves to the left by virtue of the energy stored in the spring 89. For the purpose of controlling the sequence of operations, suitable limit switches 90 and 91 are associated with the fluid motor 84. The limit switch 90 is caused to close its contacts 90a momentarily as the pusher mechanism 79 returns to the position shown in Figs. 13a and 13b of the drawings following pushing of cartridge cases 42 into tubes 36. The limit switch 91, on the other hand, is actuated just as the pusher mechanism 79 reaches the end of its stroke of inserting cartridge cases 42 into the feed end 37 of the tubes 36. At that time limit switch 91 closes its contacts 91a and opens its contacts 91b.

In Fig. 11 the operation of the pusher mechanism can readily be appreciated. One finger 80 of the pusher mechanism is illustrated as being opposite the receptacle 75 to push a cartridge case 42 contained therein out of the receptacle 75 and into the flared end 37 of a corresponding tube 36.

As far as the present invention is concerned, it is immaterial whether the cartridge cases move through the furnace open end first or base end first, the important criterion being that all of them move through the furnace orientated in exactly the same way. However, since the pusher mechanism 79 will work in a much more satisfactory manner if the fingers 80 can engage the base of the cartridge cases 42, the cartridge cases are pushed through the furnace, and specifically through the tubes 36, open end first. It will be apparent that the fingers 80 upon movement toward the roller chain conveyor 71 enter the cartridge case receptacles 75 of the magazine and engage the base of the cartridge cases disposed within these receptacles 75, thereby moving the same out of the receptacles 75 and into the tubes 36. With this arrangement the flames which exist at the feed end of each of the tubes 36 in no way interfere with the operation of supplying cartridge cases 42 to these tubes 36, since no manual operation adjacent these tubes 36 is required.

In view of the flame appearing at the ends of the tubes 36, as was mentioned above, the cartridge cases are loaded into the receptacles 75 in a loading zone to one side of the furnace 20. To accomplish this, it will be understood that the endless magazine extends to one side of the furnace 22 to a sufficient extent so that at least as many receptacles 75 as there are tubes 36 may be filled with cartridge cases, while this number of receptacles being filled are disposed to one side of the furnace proper. Movement of the roller chain 71 may be accomplished by means of any suitable prime mover. Preferably, and as illustrated in Fig. 3 and as schematically illustrated in Figs. 13a and 13b of the drawings, a suitable fluid motor 93 comprising a cylinder 94 and a piston 95 is employed. This reciprocating fluid motor 93 preferably has the piston 95 connected to a connecting rod 95a which in turn is connected between the ends of a chain 96 mounted over small diameter sprockets 97. The chain 96 and connecting rod 95a effectively define an endless chain. Reciprocal movement of the piston 95 will cause angular movement of the sprockets 97.

To operate fluid motor 93, a solenoid operated valve 92 similar to the valve 88 described above is employed as schematically indicated in Figs. 13a and 13b of the drawings. Also, a limit switch 101 is associated with fluid motor 93, which limit switch 101 has its normally closed contacts 101a opened whenever the piston 95 reaches the end of its stroke following energization of the solenoid operated valve 92.

One of the sprockets 97 is preferably connected to a shaft 98 and through a suitable one-way clutch mechanism 99 to drive one of the sprockets 72 supporting the cartridge case conveyor 71. By virtue of the one-way clutch mechanism 99, reciprocal motion of the piston 95 will cause motion in only one direction of the cartridge case magazine. Moreover, by virtue of the relative sizes of the sprockets 97 and 72, substantial motion multiplication occurs to insure with limited movement of piston 95 sufficient movement of chain 71 to cause in each cycle of movement thereof that the same number of receptacles 75 containing cartridge cases 42 therein as there are tubes 36 move into juxtaposition with the flared ends 37 of these tubes.

To make sure that the cartridge cases 42 are placed in the magazine so the open end enters the furnace first, there is provided at the loading zone a suitable loading spacer plate 100 supported immediately above the receptacles 75 at the portion of the magazine extending to one side of the furnace 20. This spacer plate 100 includes a plurality of spaced pockets 102 spaced apart the same

distance as the receptacles 75. Moreover, each pocket 102 in the magazine 100 is capable of holding a predetermined number of vertically stacked cartridge cases, four being shown by way of example in Fig. 4 of the drawings. In order to make sure that the cartridge cases 42 can only be inserted into the pockets 102 with a predetermined orientation, these pockets are of tapered configuration (somewhat like the cartridge cases 42 themselves) designated at 104 in Fig. 3 of the drawings, thus making it necessary for the base of the cartridge cases to be disposed toward the enlarged ends of the pockets 102. This affords positive assurance that all the cartridge cases 42 will be automatically inserted into the tubes 36, with the base portions thereof inserted last, thus insuring uniform heat treating. These cartridge cases can be placed into the pockets 102 manually or automatically. The spacer plate 100 is, furthermore, disposed so that when the magazine 71 stops to permit the pusher mechanism 79 to push the cartridge cases in receptacles 75 into the open ends of the tubes 36, the receptacles 75 disposed beneath the spacer plate 100 are in juxtaposition or alignment with the pocket 102 so that the cartridge cases 42 automatically fall into the open receptacles 75.

As was mentioned above, one of the important features of the hardening furnace 20 of the present invention resides in the very quick quench whereby the cartridge cases are reduced in temperature from some 1600° F. to room temperature in a matter of a few seconds. To accomplish this, there is provided in accordance with the present invention an improved quenching arrangement which is immediately adjacent the discharge end of the furnace 20 so that no delay in the quenching of the cartridge cases occurs. As best shown in Figs. 2 and 8 of the drawings, there is disposed beneath the plurality of discharge chutes 51, a different one of which is connected to different ones of the outlet ends of the tubes 36, an elongated quench liquid collecting tank 110. The particular construction of this tank 110 forms no part of the present invention. Means are preferably provided whereby liquid from tank 110 is withdrawn and cooled to a temperature of 40° F. by means not shown for subsequent reuse as a quench liquid.

For the purpose of insuring a complete and rapid quench of each cartridge case 42 to reduce its temperature from something over 1600° F. to a temperature of the order of room temperature or lower, there is provided an elongated cartridge case receiving cage 115, preferably in the form of a rectangular box extending across the discharge end of the furnace 20 and pivotally supported on the tank 110 by means of an elongated shaft 116. The cage 115 in one extreme position thereof, as shown in solid lines in the drawings, is disposed to receive cartridge cases 42 falling through chutes 51. This position is termed the cartridge case receiving position of the cage 115. The other extreme position of cage 115 shown in dotted lines in the drawings is termed the cartridge case discharge position of the cage 115. This pivotal movement of cage 115 from the cartridge case receiving position to the cartridge case discharge position is an angular movement of the order of about 120°.

It will be understood that pivotal movement of the cage 115 must occur in timed sequence with the operation of the pusher mechanism 79, so that when new cartridge cases are pushed into the tubes 36, the cage 115 is in its cartridge case receiving position to receive the cartridge cases which are pushed out of the discharge end of the tubes 36, and, furthermore, so that when the pusher mechanism 79 is inactive the cage 115 is moved to the cartridge case discharge position to discharge the quenched cartridge cases disposed therein. In view of the fact that fluid motors have already been described for performing certain control operations in connection with the present hardening furnace, a fluid motor will also be described for pivoting the cage 115, although it should be understood that any other suitable prime mover may

be employed. As best illustrated in Figs. 2, 13a and 13b, a fluid motor 120 comprising a piston 121 and a cylinder 122 is employed. The ends of a piston rod 119 of fluid motor 120 are connected to a suitable sprocket chain 119a, which chain and piston rod in effect provide an endless chain mounted on suitable sprockets 123 and 124. The sprocket 124 is illustrated as being attached to the cage shaft 116, whereupon reciprocal movement of the piston 121 will cause pivotal movement of the cage 115. 5 For the purpose of simplifying the disclosure, the fluid motor 120 is schematically indicated as of the spring return type in which a spring 126 causes return of the piston 121 after movement occasioned by supplying a hydraulic fluid to the cylinder 122 through operation of a solenoid operated valve 128. It will be understood that the solenoid operated valve 128 might just as well upon deenergization supply hydraulic fluid to the cylinder 122 to cause return movement thereof instead of employing the spring 126. Whenever solenoid operated valve 128 10 is energized, piston 121 moves to the right, as viewed in Figs. 13a and 13b, and cage 115 moves from the cartridge case receiving position shown in solid lines in the drawings to the cartridge case discharge position shown in dotted lines in the drawings.

25 In order to tie in the operation of the fluid motor 120 with the operation of the fluid motors 84 and 93, a pair of limit switches 129 and 130 are provided. The limit switch 129 is actuated to close its normally open contacts 129a and open its normally closed contacts 129b when the cage 115 reaches its cartridge case discharge or dotted line position. The limit switch 130, on the other hand, closes its contacts 130a and opens its contacts 130b when the cage 115 reaches its cartridge case receiving position, or, in other words, the solid line position shown in the 30 drawings.

To insure very high speed quench, and moreover uniform quench of the entire cartridge case as it drops into the cage 115 (such a cartridge case being shown in section and designated by the reference numeral 42 in Fig. 8 of the drawings), it is desirable to supply a quenching fluid 35 which impinges against the internal walls of the cartridge case as well as the quench jet 64 already described which impinges on the outside thereof. To this end there are supported within cage 115 a plurality of spaced internal quench tubes or nozzles 132, disposed along the longitudinal axis of the cage 115. These internal quench tubes or nozzles are arranged so that the open ends of the cartridge cases 42 slip over the tubes 132, which preferably are somewhat tapered as indicated at 133 to facilitate this action. For the purpose of guiding the cartridge cases 42 40 in their movement into the cage 115, suitable fins or guides 136 are fastened as indicated at 137 to the inside of the cage 115 at spaced points, so that a pair of guides are associated with each nozzle 132. Gravity will, of course, cause the cartridge cases to drop against the fins or guides and, hence, move over the internal quench nozzles 132 in the manner clearly indicated in Fig. 8 of the drawings.

45 It will be apparent that means should be provided to support the cartridge cases 42 above the nozzles 132 so that the base of the cartridge case does not close the nozzle, and to this end suitable support members 140 are disposed adjacent each of the nozzles 132 upon which the open end of the cartridge cases may rest. These support members are preferably fastened to the walls of the cage 115 50 as indicated at 141. The effectiveness of the quench of the present invention will readily be apparent by an examination of Fig. 8, which shows that the internal quench stream impinges against the base of the cartridge case and runs down along the inside walls of the cartridge case. Similarly, the external quench impinges against the base and runs down the exterior surface. Moreover, the cage or elongated trough 115 is provided with a limited number of openings, such as 145 in the bottom, so that it is normally full of water or quench liquid, and in fact the liquid 55

## 11

runs over the forward edge thereof as indicated in Fig. 2 of the drawings into collecting tank 110. To insure that the liquid only spills over the forward edge, the ends of the cage 115 are provided with a baffle or extension 146, best shown in Fig. 8 of the drawings. Thus, the cartridge case is subjected to an internal and external jet of cool liquid having a temperature of the order of 40° and, in addition, is completely immersed within the cool liquid. Due to the very high temperature of the cartridge case as it enters the cage 115, a rapid formation of steam occurs, and the internal and external quench jets effectively "wipe off" the steam from the surface of the cartridge case, which steam otherwise would tend to provide an insulating layer rendering the quench liquid less effective. As a matter of fact, in a device built and operated in accordance with the present invention, the cartridge cases 42 are in the quench cage 115 a matter of a few seconds, and yet the temperature thereof is reduced from something over 1600° F. to room temperature or below.

For the purpose of supplying the liquid quench to the internal quench tubes 32, there is provided a source of cooling liquid not shown which is supplied to a header 150, which header is connected by a plurality of separate tubes or conduits 151 to each of the internal quench tubes 132, there being twenty-four such tubes 132 in the event that twenty-four tubes 36 are employed in the furnace 20. In order to control the flow of the quench liquid, which, as will become apparent from the following description, must be discontinued when the cage 115 is moved to its cartridge case discharge position, there is provided a solenoid operated valve 153 for controlling the flow of fluid to all the conduits 151. In addition, a check valve 154 is provided in each of the conduits 151. The check valves 154 permit the flow of fluid through the conduits 151 only in a direction toward the cage 115. Whenever the solenoid valve 153 is energized, cooling fluid is permitted to flow to the conduits 151.

Any suitable quench liquid may be employed, although it is preferable not to use the conventional corrosive brine solution normally comprising about 10% salt. It has been discovered that by using a wetting agent, which may be purchased on the market as Aerosol OT, a dioctyl sodium sulfosuccinate compound, or in amounts of about 1% solution, the quench liquid is effectively wetter by some four times and obviously performs a much better quenching operation. The present invention, therefore, is also concerned with the use of an improved quenching liquid.

In spite of the fact that the heating operation occurs in an atmosphere which tends to reduce scaling and oxidation, it is necessary that the hardened cartridge cases be washed, and, conventionally, they are discharged from the hardening furnace to a suitable wash tank. Such tank forms no part of the present invention but is schematically indicated in Fig. 2 of the drawings by the reference numeral 160, which wash tank may include a suitable conveyor means 161 to convey the washed cartridge cases therefrom. In accordance with the present invention, when the cage 115 is disposed in the dotted line positions of the drawings, a suitable air jet is supplied through each of the internal quench nozzles 132, thereby to positively blow the particular cartridge cases disposed in the cage 115 out of the cage. To this end suitable conduits 162 are provided adjacent the open end of the cage when disposed in the cartridge case ejecting position, so that the cartridge cases are moved through the conduits 162 in the direction of the arrow shown in Fig. 2 of the drawings and into the wash tank 160.

For the purpose of supplying the necessary air jet, there is provided a suitable source of air or other gas under pressure, supplied to a header 166, and controlled by solenoid valve 167, which controls the flow through all of a plurality of conduits 168 connected to the internal quench tubes 132 through suitable check valves 169. Whenever the solenoid actuated valve 167 is energized,

## 12

air under pressure is supplied to the quench tubes 132. It will be obvious that solenoid operated valves 153 and 167 must not be simultaneously energized. Moreover, the check valves 154 will prevent air from entering the water conduits 151 when the solenoid operated valve 167 is energized, and, similarly, the check valves 169 will prevent water from entering the air conduits 168 when the solenoid actuated valve 153 is energized.

It will be understood that the hardening furnace of the present invention should not be operated unless air under a suitable pressure is available for supply to the cage 115, and hydraulic fluid under a certain pressure is available to operate the various fluid motors 84, 93 and 120. Accordingly, in the control circuits shown on Figs. 13a and 13b, pressure switches, generally designated at 170 and 171, are provided which will interrupt the power circuit in the event that either the hydraulic pressure or air pressure is below safe operating values.

In view of the detailed description included above, the operation of the present invention will readily be understood. However, this operation can better be understood by reference to the schematic control circuit shown at Figs. 13a and 13b of the drawings. In order to perform the desired control operations in a predetermined sequence, numerous elements are preferably required, such as a cycle timer generally designated by the reference numeral 180, a starting switch 181, a stop switch 182, a power supply relay 183, a pusher control relay 184, a conveyor control relay 185, a cage position control relay 186, a quench control relay 187, and a plurality of additional relays 188 and 189, the relay 188 controlling the application of control potentials from the cycle timer 180. For the purpose of providing suitable time control, a plurality of timing relays 190, 191 and 192 are provided. The timing relay 190 is in effect a cage movement time control relay and includes a pair of normally open contacts 190a which are closed instantly upon energization of relay 190. In addition, timing relay 190 includes normally closed contacts 190b and 190c which are opened following a ten-second delay after energization of timing relay 190. Additionally, timing relay 190 includes normally open contacts 190d which are closed following a five-second delay after energization of timing relay 190. Timing relay 191 is in effect a time control relay for the air injection and includes a set of normally open contacts 191a which are closed after a delay of two seconds following energization of timing relay 191. Similarly, timing relay 192 is in effect a pusher movement time control relay comprising normally open instantaneously actuated contacts 192a and normally closed six-second time delay contacts 192b.

The pusher control relay 184 includes normally open contacts 184a and 184b for controlling the energization of pusher solenoid operated valve 88. The conveyor control relay 185 includes three sets of normally open contacts 185a, 185b and 185c. The contacts 185a are effectively seal-in contacts for maintaining relay 185 energized following momentary closure of the contacts 90a of limit switch 90. The contacts 185b and 185c, on the other hand, control the energization of conveyor solenoid operated valve 92. The cage position control relay 186 includes two sets of normally open contacts 186a and 186b for controlling the energization of cage position solenoid operated valve 128. The relay 187 comprises a single set of normally closed contacts 187a which control the energization of the quench solenoid operated valve 153. The relay 188 includes a set of normally open seal-in contacts 188a which seal in relay 188 once it is energized as long as the contacts 129b of limit switch 129 are closed, or, in other words, as long as the cage 115 is not in its cartridge case ejecting position. Additionally, relay 188 includes normally closed contacts 188b and 188c which control the energization of pusher control relay 184 in response to the appli-

cation of a control voltage from cycle timer 180. The relay 189 includes a set of normally closed contacts 189a which control the energization of timing relay 190.

In order that power from a suitable source may be applied to the control system shown in Figs. 13a and 13b of the drawings, there is illustrated a source of power 193, illustrated as comprising two power lines 193a and 193b. These power lines are connected to the system through a suitable manual control switch 194 and fuses 195. In order to simplify tracing the circuits of Figs. 13a and 13b, the power lines 193a and 193b are so designated at numerous places on these figures of the drawings. The power control relay 183 normally supplies the power from source 193 to the system upon closure of the manual switch 194 and actuation of the start switch 181. Thereafter, power control relay 183 remains energized so long as the control circuit functions properly in repetitive cycles under the control of cycle timer 180. To this end power control relay 183 includes normally open contacts 183a and 183b for supplying power to the various circuits shown in Figs. 13a and 13b. Additionally, power control relay 183 includes a set of normally open seal-in contacts 183c which parallel the start button 181. Also, the relay 183 includes a set of normally closed contacts 183d for controlling the energization of a suitable signal light 199. This signal light is preferably a red signal light and when energized indicates that the switch 194 is closed but that otherwise the system is not functioning as intended. A signal light 200, which might be a green signal light, is provided, which is connected across power lines 193a and 193b through contacts 190c of timing relay 190. When this light 200 is energized, it will indicate that the system is functioning normally, and under these conditions signal light 199 will not be energized.

Before considering the operation of the control circuit, a brief description of the cycle timer 180 will first be included. Preferably this cycle timer includes a manually adjustable knob schematically indicated at 201, by means of which the length of the timing cycle can be adjustably controlled. In a particular embodiment of the present invention the cycle timer 180 was adjusted to have a cycle of twenty seconds, but obviously any other adjustment thereof may be employed. As illustrated, the cycle timer comprises a relay 202 having normally closed contacts 202a, a relay 204 having normally open contacts 204a, a motor 205 for driving a cam 206 in order to periodically close the contacts of a suitable switch having contacts 207a and 207b. A suitable manual switch 209 is included in the cycle timer 180, whereby the timer may be placed in operation upon closing switch 209. It will be apparent that the relay 202 will be energized once during each cycle of rotation of the motor driven cam 206, with the result that once during each cycle of the operation of the cycle timer, relay 204 will close its contacts 204a. These contacts control the energization circuit for the pusher control relay 184. This circuit may be traced from one line terminal 193a through the contacts 204a of relay 204, the contacts 188b of the relay 188, the conductor 212, the contacts 91b of the limit switch 91, the winding of pusher control relay 184 to line terminal 193b. It is apparent then that once during each cycle of the cycle timer 180, and if set for a twenty-second cycle, twenty seconds after manual switch 209 is closed, pusher control relay 184 will be energized to start pushing a new group of cartridge cases 42 into the tubes 36, and, consequently, pushing similar cartridge cases 42 out of the other ends of the tubes 36 and into the discharge chutes 51.

Assuming now that the control circuit is in the condition shown in Figs. 13a and 13b, upon closing of the manual switch 194 signal light 199 will be energized. The manual switch 209 of the cycle timer 180 must also be closed. If the pressure switches 170 and 171

5 are closed indicating that proper conditions exist in the system, the cycle of operation may be initiated by depressing start switch 181, with the result that power control relay 183 will be energized through a circuit from line terminal 193a through start switch 181, stop switch 182, the winding of relay 183, the six-second time delay contacts of timing relay 192, the conductor 213, the ten-second time delay contacts 190b of timing relay 190, the conductor 214, and back to the line terminal 193b. Thereupon, power control relay 183 closes its three sets of normally open contacts to supply power to the power lines 193a and 193b extending across the center of Figs. 13a and 13b and to close its seal-in contacts 183c paralleling start switch 181. It will be obvious that at any time power control relay 183 may be deenergized by manually depressing stop button 182. The signal light 199 is deenergized, and the signal light 200 is energized through the contacts 190c of timing relay 190. The reason for including the six-second time delay contacts 192b and the ten-second time delay contacts 190b in the energization circuit of power control relay 183 is one of safety, wherein power is cut off in the event that the pusher mechanism does not complete its pushing cycle in less than six seconds, or if the cage mechanism 115 does not complete its cycle in ten seconds, as will become more evident from the following description.

Following operation of power control relay 183, as determined by the cycle controlled by cycle timer 180, pusher control relay 184 will be energized with the result that solenoid operated valve 88 causes the pusher mechanism, comprising fluid motor 84, to operate and push the particular cartridge cases disposed in the magazine receptacles 75 into the tubes 36. It will be apparent that at this time the cage 115 should be in its solid line position. This is assured by virtue of the fact that the contacts 130a of limit switch 130 must be closed before solenoid operated valve 88 can be energized, and the contacts 130a of limit switch 130 are only closed when the cage 115 is in the cartridge case receiving position shown in solid lines in the drawings. During this time it should be noted that the solenoid operated valve 153 controlling the internal quench jet supplied to quench tubes 132 is energized through a circuit which may be traced from line terminal 193a, contacts 187a of relay 187, conductor 216, and the winding of solenoid operated valve 153 to line terminal 193b. It will be understood that the internal quench will be supplied as long as relay 187, which is effectively the quench control relay, is not energized.

As the fluid motor 84 is actuated to push cartridge cases 42 into the furnace, it will be noted that limit switch 90 is not actuated, since in effect it can only be momentarily energized as the fluid motor 84 substantially has completed its return stroke. However, when fluid motor 84 causes its piston 82 to move its full distance to the right as viewed in Fig. 13b of the drawings, limit switch 91 is actuated to open its contacts 91b and deenergize pusher control relay 184. It will have been noted that upon the application of a potential through the contacts 188b of relay 188 following a cycle of operation of cycle timer 180, timing relay 192 will have been energized simultaneously with pusher control 184 through the same circuit, including conductor 212, limit switch contacts 91b, conductor 217, and the winding of timing relay 192. Timing relay 192 closes its instantaneous contacts 192a, which effectively seals in its energization circuit regardless of what happens to the cycle timer 180 thereafter, and effectively connects line terminal 193a to conductor 212 through its contacts 192a and the contacts 188c of the relay 188. Timing relay 192 is deenergized simultaneously with deenergization of pusher control relay 184 upon opening of limit switch contacts 91b. Since the operation of the pusher mechanism should be accomplished in a time

somewhat of the order of three seconds, timing relay 192 should be deenergized in about three seconds. In the event that it is not deenergized within six seconds, thus indicating that the pusher mechanism is not functioning properly, contacts 192b thereof will open thereby deenergizing the energization circuit of power control relay 183, with the result that the entire system is deenergized. At the end of the forward stroke of fluid motor 84, the contacts 91a of limit switch 91 are closed thereby completing an energization circuit for timing relay 190. This circuit may be traced from power line 193a through the contacts 91a of limit switch 91, conductor 218, contacts 189a of relay 189, conductor 219, the winding of relay 190 to the power line 193b. Timing control relay 190, upon closing of its instantaneous contacts 190a, effectively seals in the energization circuit for timing relay 190 insofar as the contacts 91a of the limit switch 91 are concerned, whereby these contacts 91a may be reopened upon the return stroke of fluid motor 84 without deenergizing timing relay 190. The instantaneous contacts 190a of timing relay 190 also complete the energization circuit of relay 188. This circuit may be traced from line terminal 193b through the winding of relay 188, conductor 218, contacts 190a of timing relay 190 to line terminal 193a. The energization of relay 188 causes closing of its contacts 188a, which effectively seal in relay 188 through contacts 129b of limit switch 129. This circuit can be traced from power line 193a, contacts 129b of limit switch 129, conductor 220, contacts 188a of relay 188, and the winding of relay 188 to power line 193b. Upon a delay of five seconds following energization of timing relay 190, its five-second time delay contacts 190 close, thus assuring that the cage 115 will remain in the solid line position shown for at least five seconds, during which time cartridge cases are dropped into the cage and subjected to the internal and external quench mentioned above. Upon closure of the five-second delay contacts 190d, cage position control relay 186 is energized through an obvious circuit to cause solenoid operated valve 128 to be energized, whereupon the fluid motor 120 causes cage 115 to move from its solid line position to its cartridge case ejecting position shown in dotted lines in the drawings. As the cage starts to move about its shaft 116 (clockwise as viewed in Fig. 13b of the drawings), the contacts 130b of limit switch 130 are closed, and, similarly, the contacts 130a of this limit switch are open, the latter contacts making sure that the pusher mechanism cannot be actuated unless the cage 115 is in its cartridge case receiving position. Closure of contacts 130b energizes quench control relay 187 through a circuit which may be traced from line 193a through contacts 130b, through conductor 221, and through the winding of relay 187 to power line 193b. Energization of quench control relay 187 opens contacts 187a to deenergize the quench control solenoid operated valve 153, thus cutting off the internal quench jets while the cage is moving to its cartridge case ejecting position. As the cage 115 reaches its cartridge case ejecting position, limit switch 129 is actuated to close its contacts 129a and open its contacts 129b. Closing of the contacts 129a causes simultaneous energization of the air ejection solenoid operated valve 167 and timing relay 191. This circuit can be traced from power line 193a through contacts 129a, through conductor 222, through the winding of the relay 191, to power line 193b or to the winding of solenoid operated valve 167, which latter two windings are in parallel. Thus, an air jet is supplied through the internal quench nozzles 132 to eject the cartridge cases disposed within the cage 115. This air injection is permitted to exist for a period of two the winding, controlled by the two-second delay contacts 191a of timing relay 191. At the end of this two-second period these contacts 191a are closed to complete

an energization circuit for the relay 189 through an obvious circuit. When relay 189 opens its contacts 189a there occurs the resultant deenergization of timing relay 190. In the event that more than ten seconds have elapsed between the time that timing relay 190 is energized and the time it is deenergized through the energization of relay 189, the ten-second delay contacts 190b of timing relay 190 will interrupt the energization circuit for power control relay 183 and shut down the system. This will only occur if the cage 115 does not complete its cycle within a ten-second period. Actually, it should complete its cycle in around seven seconds. It will be observed that when the cage 115 reaches its cage ejection position, limit switch contacts 129b are opened to break the energization circuit for relay 188 through these contacts, and upon deenergization of timing relay 190 relay 188 opens to permit a subsequent control voltage from cycle timer 180 to initiate a subsequent cycle of operation. Quench control relay 187 is also deenergized as soon as cage 115 reaches its cage receiving position, whereupon the internal quench jets are again turned on through energization of solenoid operated valve 153.

It will be apparent that during the cycle just described, the fluid motor 93 must be energized to move a new charge of cartridge cases 42 disposed within receptacles 75 in the magazine into a position for actuation by fingers 80 to move the same into the tubes 36. Thus, upon momentary closure of limit switch 90, which only occurs when the fluid motor 84 has almost completed its return stroke, the conveyor control solenoid 185 is energized. This circuit can be traced from power line 193b through the winding of relay 185, the contacts 101a of the limit switch 101, and the contacts 90a of the limit switch 90 to power line 193a. Conveyor control relay 185 includes seal-in contacts 105a paralleling the contacts 90a of limit switch 90 which are only momentarily energized. Upon energization of conveyor control relay 185, solenoid operated valve 92 is energized to cause fluid motor 93 to rotate the magazine forward, so that twenty-four different receptacles 75 are moved opposite the ends of the twenty-four tubes 36 of the furnace 20. Upon completing its forward stroke, fluid motor 93 actuates limit switch 101 to open its contacts 101a and deenergize conveyor control relay 185 and, hence, solenoid operated valve 92, whereby fluid motor 93 is returned by means not shown to its initial operating position for a subsequent conveyor operation.

It will be apparent that as cycle timer 180 causes its contacts 204a to be closed again, the entire operation just described will be repeated.

The furnace of the present invention is normally operated on a continuous shift basis, since shutting down the furnace causes complications with reference to scaling and the like of cartridge cases disposed within the tubes 36. However, since it is contemplated that the furnace 20 be shut down, it is preferable that the tubes 36 be charged with rejected cartridge cases so that they can be thrown away when they are subsequently pushed through the furnace, since the inordinate amount of scaling which will occur makes these cartridge cases unacceptable if they were otherwise acceptable. Hence, on week-ends or on days preceding holidays, the operators prior to shutting down the furnace will fill the tubes 36 with rejected cartridge cases. Also upon subsequently starting up the furnace cam 58 will make sure that if there has been any welding which has not been disturbed by the protuberances 46, that this weld is broken.

Although there has been described an arrangement in which a plurality of individual tubes 36 are employed in the furnace 20, a somewhat simplified construction is illustrated in Figs. 14 and 15 of the drawings, in which a pair of cooperating somewhat corrugated-like plates 230 and 231 provide a plurality of connected passageways

similar to the individual tubes 36. The individual passageways are designated by the reference numeral 232, and they have the same V-shaped cross section to provide for better distribution of the weight of the cartridge cases, thus eliminating deformation of the cartridge cases. Also, instead of having a controlled atmosphere only within the passageways 232, the entire heating chamber 22 of the furnace is supplied with a nonoxidizing atmosphere. The same protuberances designated as 233 in Fig. 15 of the drawings are employed as those designated by the reference numeral 46 and perform exactly the same function. It will be understood that as far as supporting the cartridge cases in their movement through the furnace is concerned the upper plate 230 is not essential. However, a considerable force must be transmitted by each cartridge case, and this force is at a maximum for the particular cartridge cases which are just being inserted into the furnace, and decreases gradually as the cartridge cases move along the furnace, due to the fact that there are less cartridge cases ahead of them to be pushed along. The top plate 230 prevents the cartridge cases from tipping up under the large forces which might be involved for the cartridge cases near the entrance of the furnace. However, it has been found that this top plate 230 is not necessary throughout the entire furnace, and, as illustrated in Fig. 15, extends only part way through the furnace. The operation of the arrangement shown in Figs. 14 and 15 will be readily apparent to those skilled in the art.

While there has been illustrated and described an improved system, apparatus and process for hardening steel cartridge cases, it will be apparent to those skilled in the art that numerous changes and modifications will occur, and it is aimed in the appended claims to cover all such changes and modifications as fall within the true spirit and scope of the present invention.

What is claimed as new and desired to be secured by Letters Patent of the United States is:

1. Apparatus for hardening cartridge cases comprising a high temperature heating chamber, means defining a tubular passageway through said heating chamber through which said cartridge cases may be moved in end-to-end relationship with every case orientated in the same way, means in said tubular passageway located at spaced points therealong for causing relative transverse movement of adjacent cases to cause relative movement between the engaging ends of said cases, a discharge chute connected to one end of said tubular passageway through which said cartridge cases fall upon being moved out of said end of said passageway, cartridge case engaging means at the junction of said passageway and discharge chute for deflecting said cases into said discharge chute in the event that they fail to fall by gravity into said chute upon movement out of said passageway, and means for inserting cartridge cases into the other end of said passageway and simultaneously pushing cases disposed in said passageway along said passageway.

2. A quenching means for rapidly cooling work pieces in the form of a tube closed at one end which have been subjected to high temperatures comprising a movable receptacle for receiving said work pieces to be quenched, means for subjecting said work pieces to internal and external jets of quenching liquid while disposed in said receptacle, means for terminating said internal jet after a predetermined time delay, means for moving said receptacle to a work piece discharge position, and means for supplying a blast of fluid into the interior of each work piece while in said receptacle and while said receptacle is in its work piece discharge position for ejecting said work piece from said receptacle.

3. A hardening furnace for work pieces comprising a heating chamber within which temperatures in excess of 1600° F. may be obtained, means defining a passageway through said heating chamber through which said work

pieces may be moved in end-to-end relationship with every work piece orientated in the same way, means for inserting work pieces into one end of said passageway and simultaneously pushing work pieces disposed in said passageway along said passageway, means for receiving said work pieces in a first predetermined position as they are being pushed out of the other end of said passageway, means correlated with the operation of the work piece inserting means for moving the receiving means to a second predetermined position, means for subjecting said work pieces to a liquid quench when the receiving means is disposed in said first predetermined position, means for terminating the operation of the last mentioned means during the movement of the receiving means to said second predetermined position, and means for discharging said work pieces from said means for receiving the same following movement to said second predetermined position.

4. A hardening furnace for work pieces comprising a heating chamber within which temperatures in excess of 1600° F. may be obtained, means defining a passageway through said heating chamber through which said work pieces may be moved in end-to-end relationship with every work piece orientated in the same way, means for inserting work pieces into one end of said passageway and simultaneously pushing work pieces disposed in said passageway along said passageway, means for receiving said work pieces upon being pushed out of the other end of said passageway, intermittently operated means for subjecting said work pieces to a liquid quench when disposed in said last mentioned means, means correlated with the operation of said work piece inserting means for actuating said last named means, means for discharging said work pieces from said means for receiving the same following rapid quenching thereof, and a movable magazine operated in timed relation with respect to the discharge means and the work piece inserting means for moving work pieces adjacent to said one end of the passageway whereby said means for inserting work pieces may move them out of said magazine and into said one end of said passageway.

5. A hardening furnace for work pieces comprising a heating chamber, means defining a passageway through said heating chamber through which said work pieces may be moved in end-to-end relationship with every work piece orientated in the same way, means for inserting work pieces into one end of said passageway and simultaneously pushing work pieces disposed in said passageway along said passageway, a discharge chute connected to the other end of said tubular passageway through which said work pieces fall upon being moved out of said other end of said passageway, a pivotally mounted receptacle disposed beneath said discharge chute and capable of receiving said work pieces dropping through said discharge chute when disposed in one predetermined position, means for subjecting said work pieces to a liquid quench while said receptacle is disposed in said one predetermined position, means operated in timed relation with respect to the work piece inserting means for pivoting said receptacle to a different predetermined position and terminating said liquid quench at least before the end of the period of said pivoting of said receptacle, and air jet means operable in timed relation with respect to the operation of the pivoting means for removing said work pieces from said receptacle while disposed in said different predetermined position.

6. In a hardening furnace for cartridge cases comprising a heating chamber, means defining a passageway through said heating chamber through which said cartridge cases may be moved in end-to-end relationship with every cartridge case orientated in the same way, a movable endless belt magazine into which said cartridge cases are placed, means for moving said cartridge cases out of said magazine and into one end of said passageway and simultaneously pushing cartridge cases disposed in

said passageway along said passageway, a discharge chute connected to the other end of said tubular passageway through which said cartridge cases fall upon being moved out of said other end of said passageway, a pivotally mounted receptacle disposed beneath said discharge chute and capable of receiving said cartridge cases dropping through said discharge chute when disposed in one predetermined position, means for subjecting said cartridge cases to a liquid quench while said receptacle is disposed in said one predetermined position, means operated in 10 timed relation with the operation of the work piece inserting means for pivoting said receptacle to a different predetermined position, and air jet means operated in timed relation with respect to the movement of the pivoting means for removing said cartridge cases from said receptacle while disposed in said different predetermined position.

7. A quenching means for rapidly cooling cartridge cases which have been subjected to temperatures above 1000° F. to room temperature or below in a few seconds, comprising a movable receptacle for receiving said cases to be quenched, means for subjecting said cases to an external stream of quenching liquid while disposed in said receptacle, an internal quench tube for supplying a jet of quenching liquid to the interior of each cartridge case, means for terminating said internal jet after a predetermined time delay, means for moving said receptacle to a cartridge case discharge position, and means for supplying a blast of air through said quench tube to the interior of such cases while in said receptacle and while said receptacle is in its discharge position for ejecting said cartridge cases therefrom.

8. The method of cooling a tubular work piece closed at one end which has been heated to a high temperature of the order of 1600° F. to room temperature or below in a period of a few seconds which comprises dropping said heated work piece open end first through a wall of quenching liquid at a temperature well below room temperature, momentarily supporting said work piece immediately below said wall of quenching liquid so the exterior thereof is still subjected to cooling thereby, applying a jet of said liquid against the interior walls of said work piece momentarily supported below said wall of quenching liquid, terminating said liquid jet, and subjecting the interior of said work piece to a blast of air to displace said work piece from its position of momentary support immediately below said liquid wall.

9. The method of cooling a cartridge case which has been heated to a high temperature above 1000° F. to room temperature or below in a period of a few seconds, which comprises dropping said cartridge case open end first through a conical shaped wall of quenching liquid at a temperature well below room temperature, momentarily supporting said work piece immediately below said wall of quenching liquid so the apex of said conical wall strikes the base of said case and subjects the exterior thereof to cooling thereby, applying a jet of said liquid against the interior of said cartridge case while momentarily supported below said wall of quenching liquid, terminating said liquid jet, and supplying a blast of air to the interior of said cartridge case to displace it from its position of momentary support immediately below said liquid wall.

10. A hardening furnace for work pieces comprising 65 a heating chamber having a passageway therein through which work pieces may be moved in end to end relationship, said passageway having entrance and discharge ends, loading means for inserting work pieces into the entrance end of said passageway and simultaneously pushing work pieces disposed in said passageway there-through in order to discharge work pieces from the discharge end of said passageway, quenching means posi-

5 tioned adjacent the discharge end of said discharge passageway for directing a jet of quenching liquid onto each of said work pieces as it emerges from the discharge end of said passageway, and means correlated with the operation of said loading means for intermittently operating said quenching means to cut off the jet for predetermined intervals during the period between the emergence of successive work pieces from the discharge end of said passageway.

11. A hardening furnace for work pieces comprising a 10 heating chamber having a passageway therein through which work pieces may be moved in end to end relationship, said passageway having entrance and discharge ends, loading means for inserting work pieces into the entrance end of said passageway and simultaneously pushing work pieces disposed in said passageway therethrough in order to discharge work pieces from the discharge end of said passageway, quenching means positioned adjacent the discharge end of said discharge passageway for directing a jet of quenching liquid onto each of said work pieces as it emerges from the discharge end of said passageway, means operated in timed relation with respect to said loading means for intermittently rendering said quenching means operative for a predetermined interval after 15 one of said work pieces is moved out of the discharge end of said passageway, and means for rendering said quenching means inoperative at the termination of said predetermined interval thereby cutting off the jet.

12. A hardening furnace comprising a heating chamber for work pieces including a passageway having entrance and discharge ends, loading means for moving work pieces through said passageway to the discharge end thereof, a movable magazine for moving said work pieces to a position adjacent to the entrance end of said 20 passageway from which the loading means may move them into the entrance end of said passageway, means responsive to the actuation of said loading means for operating said moveable magazine, means for receiving each individual work piece discharged from the discharge 25 end of said passageway, means for subjecting said work piece to a liquid quench while disposed in the receiving means, means for removing the work piece from said receiving means after it is quenched, means for moving said receiving means from its receiving position to a work 30 piece removing position and for returning the receiving means to its receiving position, means for rendering the removing means operative when the receiving means is in said removing position, and means for rendering the loading means operative as soon as the receiving means 35 is returned to its receiving position and for preventing the operation of said loading means until the receiving means is in said receiving position.

#### References Cited in the file of this patent

#### UNITED STATES PATENTS

|           |                     |                |
|-----------|---------------------|----------------|
| 519,232   | Brustlein           | May 1, 1894    |
| 1,227,027 | Baily et al.        | May 22, 1917   |
| 1,866,806 | Holly               | July 12, 1932  |
| 1,888,960 | Talley              | Nov. 22, 1932  |
| 1,957,932 | Beroizheimer et al. | May 8, 1934    |
| 2,063,784 | Becktel et al.      | Dec. 8, 1936   |
| 2,235,542 | Wenzel              | Mar. 18, 1941  |
| 2,298,149 | Morton              | Oct. 6, 1942   |
| 2,325,757 | Ehlers              | Aug. 3, 1943   |
| 2,352,709 | Haase               | July 4, 1944   |
| 2,450,112 | Buckholdt           | Sept. 28, 1948 |
| 2,462,851 | Fawcett             | Mar. 1, 1949   |
| 2,583,046 | Gardner             | Jan. 22, 1952  |

#### FOREIGN PATENTS

|         |               |               |
|---------|---------------|---------------|
| 352,174 | Great Britain | July 9, 1931  |
| 532,807 | Great Britain | Jan. 31, 1941 |